

No. 869,870.

PATENTED NOV. 5, 1907.

M. AMS.  
COMPOSITION OF MATTER.  
APPLICATION FILED FEB. 8, 1907.

Fig. 1.



Fig. 2.



WITNESSES

James F. Duhamel  
Frank L.

INVENTOR

Mark Ams  
BY  
W. F. Gourieau  
ATTORNEY.

# UNITED STATES PATENT OFFICE.

MAX AMS, OF NEW YORK, N. Y., ASSIGNOR TO CHARLES M. AMS, OF NEW YORK, N. Y.

## COMPOSITION OF MATTER.

No. 869,870.

Specification of Letters Patent.

Patented Nov. 5, 1907.

Application filed February 8, 1907. Serial No. 356,443.

*To all whom it may concern:*

Be it known that I, MAX AMS, a citizen of the United States, and a resident of the city of New York, in the county and State of New York, have invented certain 5 new and useful Composition of Matter, of which the following is a specification.

This invention relates to a composition of matter to serve as a packing to insure the hermetic sealing of sheet-metal containers, known in general parlance as 10 "tin cans," in which the separate parts of the can-body are secured to each other by what is known as the seaming or double-seaming process, without the employment of solder or other form of metallic cement.

Of course, where the parts of the can are soldered 15 together in the old way, the solder, as well as uniting the parts together, at the same time naturally effects a hermetically-tight joint. In the more modern process of double-seaming, designed, among other things, to eliminate the use of solder, overlying layers of the 20 edges of parts of the container designed to be secured together, are rolled or folded and pressed together to make an interlocking joint, which forms what may be termed a bead, comprising portions of both parts. Such a joint might possibly be made "air tight" with 25 out other process or adjunct; but in the rapid manufacture and sealing of such cans by machinery, for commercial purposes, it is impracticable, of course, if not impossible, to give each can such individual attention as would be necessary to insure perfect sealing. I have 30 found it most desirable, therefore, to coat one or the other of the two contacting surfaces which are to be subsequently rolled or folded together, with a composition or material primarily for the purpose of forming a yielding seat which will compensate for slight 35 irregularities in one or the other of said parts or in the operation of a machine designed to join the same.

While this is the more important function of such a material or composition, there are a number of other properties which it should possess, and which must be 40 taken into consideration. In the first place, the employment of a separate packing ring is objectionable for many reasons, not least among which is the excessive amount of material required for a packing in this form and the inconvenience of handling and applying 45 such a ring in the rapid sealing of cans by machinery. This packing should, therefore, be in the form of a coating upon one of the parts, and as a coating the composition, in its original state, must be adhesive, and furthermore, of a nature to adhere to tin, it being well 50 known that the nature of tin plate is such that the more common forms of adhesive substances will not of themselves adhere thereto. Furthermore, it is desirable that this substance or composition, when applied to one or the other of said parts, should have substantially 55 what is known as a "hard finish," particularly in order that the particular part coated may be handled

and manipulated independently without injury to the coating. Furthermore, while such hard finish is desirable, the applied composition should be to a certain degree plastic and flexible in order to perform 60 its primary function, as hereinbefore set forth. Moreover, the necessarily inherent qualities of such a composition make it necessary that it be composed, to a greater or less extent, of organic matter, which, as is well known, is in most cases normally subject to decomposition, or at least to deterioration as a useful agent upon long exposure. Inasmuch as the separate parts of the can are each the subject of independent manufacture, and particularly in the case of tops designed to be secured to the body portion of the can 70 after the latter has been filled with the particular form of product which it is designed to contain, such parts are frequently retained in their unjoined or separate condition for a comparatively long period of time, it is desirable that this substance or composition be proof against mold or other form of chemical change which would result in deterioration of the substance or impairment of its various properties. Furthermore, such a composition as the one in mind is likely to be and frequently is colorless when including 75 no other ingredients than those necessary to give it the qualities hereinbefore suggested, and therefore when applied to one or the other of the parts to be joined provides no means of easy and ready distinction between coated and uncoated parts of the same form. 80 Such composition should therefore be of a decided and distinctive color. Lastly, it is desirable that the ingredients which enter into the composition, each contributing to provide a number of desirable properties, should be of such character and subjected to such 85 process or treatment that they will combine to form a homogeneous mass, capable of easy handling and application, and each component substance non-interferent with the qualities of another or others.

For such a composition I have found that the concrete organic substance known as gelatin provides the best base. Gelatin in itself, however, while forming the body of the substance I have in mind and contributing to provide a suitably firm yet yielding packing which when placed between metal sheets in the manner suggested compensates for irregularities of the metal and minor imperfections in the machinery employed, requires to be combined with other ingredients, in order to provide a composition which will possess one or more of the other desirable qualities hereinbefore referred to. I have found, however, that gelatin first dissolved in water, and preferably rain water, to a proper degree of consistency, to which is added a small amount of tartaric acid, will thereby acquire a higher degree of viscosity, or stickiness, and will cause the 105 gelatinous substance to adhere to the part designed to be coated and to sufficiently retain these properties to 110

similarly adhere to the part against which the coated part is intended to be placed for the folding or rolling of the superposed layers. I have furthermore found that the addition of a small amount of formic acid will give to this coating, when applied, the so-called "hard finish," the desirable qualities of which I have hereinbefore referred to. I have furthermore found that the addition of a small amount of glycerin will tend to preserve the composition, when applied, in a soft and pliable condition, whereby the desirable yielding and elastic qualities are not impaired through the evaporation of the water after application. I have furthermore found that the addition of substantially a trace of sulfuric acid will act as a preservative and prevent deterioration or impairment of the properties of the composition through any form of decomposition, such as molding or other undesirable chemical change. While any coloring matter as a substance not antagonistic to the properties of the other ingredients may obviously be employed, I prefer the use of burnt sienna for this purpose.

In the production of this composition, and referring to a substance which includes all of the ingredients above mentioned, or the equivalents thereof, I first dissolve the gelatin in warm water, care being taken not to impair the properties of the former by raising the water to too high a temperature, much less boiling, and then add to the semifluid mass produced the ingredients referred to in preferably the order mentioned. I have found that in any given quantity of my composition, where all of the ingredients mentioned are included, that the proportion of each should, for best results, be substantially as follows:

|    |                    |                    |
|----|--------------------|--------------------|
| 35 | Rain water.....    | 66 per cent.       |
| 35 | Gelatin.....       | 30 " "             |
|    | Tartaric acid..... | 1 " "              |
|    | Formic acid.....   | $\frac{3}{4}$ " "  |
|    | Sulfuric acid..... | $\frac{1}{8}$ " "  |
| 40 | Glycerin.....      | 1 " "              |
| 40 | Burnt sienna.....  | $1\frac{1}{2}$ " " |
|    |                    | 100                |

It will be apparent that for some purposes certain of the ingredients mentioned above may be dispensed with; for instance, if the composition is to be applied and, the seaming or sealing process immediately follow, there would not be the same necessity for including a preservative, either for the inherent chemical nature of the composition or for its substantive qualities. Under some circumstances the gelatin itself might be found to possess sufficient viscosity or "stickiness" to make the addition of tartaric acid unnecessary. The coloring matter, of course, is not necessary—being merely added for convenience, to which, however, it largely contributes. There are, therefore, a number of sub-combinations of ingredients, each constituting a useful composition. In general, however, where this composition is to be made up in large quantities for subsequent use, and the can-parts themselves stored for some time prior to the sealing operation, it will be found desirable to have present in the composition all of the elements hereinbefore set forth.

Where this composition is made up for subsequent

use, the effects of evaporation will generally leave it in condition which unfit it for immediate application and use, but it may always be brought to proper or ready-to-use condition by gently heating, preferably by direct application of steam, where steam is available. It may then be applied to the can-covers or other parts through the medium of a brush, if applied by hand, or in any other desired manner by hand or machinery.

In order to illustrate the manner in which my composition is preferably used and applied I have shown in the accompanying drawings, forming a part of this specification, certain views, of which

Figure 1 is a plan-view of the end-portion or member of a cylindrical sheet-metal container to which such a coating as the one hereinbefore described has been applied, and Fig. 2 is a central sectional view of two parts designed to be secured together, illustrating the function and location of my packing when applied to a container of this style.

In these drawings I have shown the coating 3 applied in the form of an annular ring upon the top or bottom member 4 of the can-body, against which 85 coated portion the flange 5 of the body-portion 6 of the can-body is pressed for the seaming operation. It will be obvious that these illustrations are merely illustrative of one of many ways of utilizing the composition hereinbefore described, it being obvious that the can-body 90 may be of any desired configuration and that the coating may with equally satisfactory results be applied to either of the two members designed to be secured together.

Having thus described my invention, I claim as new 95 and desire to secure by Letters Patent:

1. A composition consisting of gelatin and tartaric acid, for the purpose set forth.
2. A composition consisting of a comparatively large proportion of diluted gelatin and a comparatively small 100 proportion of tartaric acid, for the purpose set forth.
3. A composition consisting of gelatin, tartaric acid and a preservative, for the purpose set forth.
4. A composition consisting of gelatin, tartaric acid and glycerin, for the purpose set forth.
5. A composition consisting of gelatin, tartaric acid and a surface-hardening agent, for the purpose set forth.
6. A composition consisting of gelatin, tartaric acid and formic acid, for the purpose set forth.
7. A composition consisting of gelatin, tartaric acid, a 110 surface-hardening agent and a physical preservative, for the purpose set forth.
8. A composition consisting of gelatin, tartaric acid, glycerin and a surface-hardening agent, for the purpose set forth.
9. A composition consisting of gelatin, tartaric acid, formic acid, and glycerin, for the purpose set forth.
10. A composition consisting of a comparatively large proportion of diluted gelatin and comparatively small proportions of tartaric acid, formic acid and glycerin, for the purpose set forth.
11. A composition consisting of gelatin, tartaric acid, a surface-hardening agent, a preservative, and a coloring agent, for the purpose set forth.
12. A composition consisting of gelatin, tartaric acid, formic acid, and a preservative, for the purpose set forth.
13. A composition consisting of gelatin, tartaric acid, formic acid, and both chemical and physical preserving agents, for the purpose set forth.
14. A composition consisting of gelatin, tartaric acid, formic acid, suitable preservative agents, and a coloring agent, for the purpose set forth.

15. A composition consisting of gelatin, tartaric acid, formic acid, glycerin, sulfuric acid, and a coloring agent, for the purpose set forth. 15
16. A composition consisting of a comparatively large proportion of diluted gelatin and comparatively small proportions of tartaric acid, formic acid, glycerin and sulfuric acid, for the purpose set forth. 20
17. A composition consisting of a comparatively large proportion of gelatin, comparatively small proportions of tartaric acid, formic acid, glycerin and sulfuric acid, and a coloring agent, for the purpose set forth. 10
18. A composition comprising the following ingredients in substantially the proportions stated: water 66 parts; gelatin 30 parts; tartaric acid, 1 part; formic acid,  $\frac{1}{2}$  part; sulfuric acid,  $\frac{1}{2}$  part; glycerin, 1 part; coloring agent  $1\frac{1}{2}$  parts; for the purpose set forth.

In testimony of the foregoing, I have hereunto set my hand in the presence of two witnesses.

MAX AMS.

Witnesses:

JOHN A. FILSNER,  
F. WEBER.